

FIP8309 XR 1,034,658  
CATION OF TEXTILES & FIBERS

## UNITED STATES PATENT OFFICE.

EDUARD STEIGER, OF ST. GALLEN, SWITZERLAND.

## METHOD OF BLEACHING.

403  
4081  
1,034,658.

Specification of Letters Patent. Patented Aug. 6, 1912.

No Drawing.

Application filed January 6, 1911. Serial No. 601,174.

*To all whom it may concern:*

Be it known that I, EDUARD STEIGER, a citizen of the Republic of Switzerland, residing at Villa Kleinberg No. 3; St. Gallen, Switzerland, have invented new and useful Improvements in Methods of Bleaching; and I do hereby declare the following to be a full, clear, and exact description of the invention, such as will enable others skilled in the art to which it appertains to make and use the same.

This invention relates to a new and improved method of completely bleaching cotton and linen yarns, tissues, embroideries, etc.

The improved method consists of a series of operations viz. a preliminary treatment by which the fats and oils and where necessary, the dressing are removed and the bleaching proper by a slightly acid bath of permanganate which is followed by a bath of soda and means for preventing yellowing of the ware through overbleaching.

As is known it was attempted hitherto to remove the fats and oils contained in the cotton or linen yarns to be bleached by means of the bucking process. This process consists in boiling the ware under pressure and for a considerable time in a caustic lye. By this operation which is as expensive as it is tedious only saponifiable vegetable or animal fats are changed into compositions which can be dissolved in water and thereby removed. But when the ware contains non-saponifiable fats, such as hydrocarbons, mineral oils or paraffins these are not dissolved and therefore remain in the merchandise wholly or partly. Such merchandise which is not perfectly free from all fatty substances has a tendency to yellow later on in consequence of the action of the fatty matter which has not been removed. This yellowing may cause great damage, for the value of a textile merchandise which is even only partly yellowed is considered to be very much reduced.

Extracting the fatty substance has the object of completely removing all fatty substances, also the non-saponifiable ones, from the yarns, tissues and embroideries to be

bleached and at the same time to obtain these fatty substances as by-products. With this object in view the yarns, tissues or embroideries are extracted with a solvent for fats and hydrocarbons in a suitable apparatus such as a Soxhlet siphon apparatus, and thus all fatty matter is removed from them. As solvents for the fatty matter petroleum ether or benzine, chlorid of ethylene, carbon tetrachlorid or mixtures of these extracting means may be employed. Cotton or linen merchandise which in the manner indicated has been carefully freed from all fatty matter may, after the dressing has been removed, be subjected to a bleaching process with the result that this process is much shorter than it was hitherto and that the tedious bucking process and the use of soap are entirely done away with. This latter circumstance has the further advantage that the difficulties adhering to the use of lime soap for the bleaching are eliminated, for it is known that often yellowing is caused by lime soap remaining in the merchandise.

The extraction of fatty matter has the following main advantages: It renders possible the removal of fatty matter to any desired degree in a short time and thus prevents yellowing through remaining fatty matter; it has the advantage that no more consideration will have to be had of the nature of the fats contained in the merchandise. For example in the case of embroideries manufactured on machines lubricated with mineral oil it may occur that some oil adheres to the ware. As this oil is non saponifiable it remained in the ware when the latter was bleached by the so called English bleaching process, and the consequence was that the ware yellowed and was spoiled. With the new process this cannot occur, because it is entirely irrelevant whether the merchandise to be bleached contains saponifiable, vegetable or animal fats or paraffins in greater or smaller quantities.

For removing the dressing, the ware, after the fatty matter has been removed, is put into a solution of diastase which has a temperature of about 50 to 65 centigrade. This

temperature must be maintained during the treatment. Diastase changes the dressing into a substance soluble in water. The reaction may be considered to be completed 5 when the ware does not show a blue tint when touched with a solution of iodin. Then the merchandise is taken from the solution of diastase and thoroughly washed. Diastase may be prepared from brewery or 10 distillery malt in the form of an aqueous extract. Using diastase for removing the dressing is very rational, particularly when large quantities have to be removed. This 15 preliminary step of the process is followed by the bleaching process proper by which operation the coloring matter is destroyed, the greatest possible care being taken of the fibers and the cellulose forming them.

20 The merchandise free from fat and dressing is treated for about two minutes with a slightly acid water solution of permanganate at the ordinary air temperature. Acetic acid is preferably used. Permanganates have been previously used for bleaching jute, but cannot be used without difficulty for cotton because cotton and jute react differently. It is desirable to use permanganate for cotton also because it bleaches 25 rapidly.

30 After treating the material to be bleached with a diluted and slightly acid solution of permanganate it is washed in water and the manganese dioxid deposited on the fiber 35 is removed by treatment with sulfurous acid or peroxid of hydrogen. When sulfurous acid is employed its concentration should be about 1 to 2° Bé. This treatment is followed by a treatment with reagents 40 having a hydrating and at the same time dissolving action on the products of decomposition of the cellulose (if these are present). Such reagents are acid lyes, but these would damage the fiber because the cellulose 45 of it would be too much affected and the strength of the fiber reduced. To overcome this drawback, that is to lastingly bleach the natural coloring matter of the cotton without damaging the fiber a diluted hot 50 solution of soda is employed the concentration of which is preferably 1° Bé. The treatment in the soda bath can be effected with or without pressure. The soda bath may also with advantage be used immediately after the treatment with permanganate and washing with water instead of at 55 the end of the series treatment. In this case the dissolving effect on the products of decomposition of the cellulose is particularly favored. Obviously a bath of potash 60 has the same effect as a soda bath.

The bleaching operations proper must be repeated several times in the succession described. After having been treated four

times, the merchandise will as a rule be completely bleached.

The last step of the process has the object of removing the products of the decomposition of cellulose (if any). At the same time the bleaching is, so to speak, completed, 70 and yellowing is prevented. For that purpose the bleached merchandise is heated in an alkaline solution of a copper salt (Fehling solution diluted with double its quantity of water) then the merchandise is removed to a solution of hydrochloric acid or sulfuric acid, and finally a solution of soda is applied.

Merchandise cotton and linen yarns, tissues, embroideries, etc., are not in danger of 80 being yellowed by fatty matters remaining in them.

Having now particularly described and ascertained the nature of the said invention and in what manner the same is to be performed, I declare that what I claim is:

1. The process of treating textiles comprising a preliminary treatment for removing the fat, bleaching chiefly with permanganate, then subjecting the product to a hot soda bath, washing it, and then finishing by treating it with an alkaline solution of copper salt, a solution of an acid, and thereafter with a solution of soda, substantially as described. 95

2. The process of treating textiles, comprising a preliminary treatment for removing the fat by means of a solvent for fats and hydrocarbons to prevent yellowing by any remaining fatty matter, bleaching 10 chiefly with permanganate, then subjecting the product to the action of a hot soda bath, washing it, and finishing by treating it with an alkaline solution of a copper salt, a solution of an acid, and thereafter with a solution of soda, substantially as described. 10

3. The process of treating textiles comprising a preliminary treatment for removing the fat from the textile product by means of a solvent for fats and hydrocarbons for the purpose of preventing yellowing by any remaining fatty matter, a treatment with a slightly diluted acid bath of permanganate, removing any dioxid of manganese deposited on the fiber, subjecting the 11 textile to a hot alkaline bath and to a finishing treatment with an alkaline solution of a copper salt, a solution of an acid, and thereafter with a solution of soda, substantially as described. 11

4. The process of bleaching textiles, comprising a preliminary treatment for removing the fat from the textile product by a solvent for fats and hydrocarbons, a treatment with a diluted, slightly acid solution 1 of permanganate; removing the superoxid deposited on the fiber, then treating the textile with a hot bath of an alkali, and subject-

ing the textile to a finishing treatment, comprising heating the textile in an alkaline solution of a copper salt, removing any remaining copper compounds with a solution of an acid and then treating the textile with a solution of soda, substantially as described.

In testimony that I claim the foregoing

as my invention, I have signed my name in presence of two subscribing witnesses.

EDUARD STEIGER

Witnesses:

ERNST FISCHER,  
CARL GUBLER.